

# UNITED STATES PATENT OFFICE.

JOHN L. COX, OF PHILADELPHIA, PENNSYLVANIA, ASSIGNOR TO MIDVALE STEEL & ORDNANCE COMPANY, OF PHILADELPHIA, PENNSYLVANIA, A CORPORATION OF DELAWARE.

## CHROMIUM-STEEL ALLOY.

1,333,654.

Specification of Letters Patent. Patented Mar. 16, 1920.

No Drawing.

Application filed May 1, 1919. Serial No. 293,964.

To all whom it may concern:

Be it known that I, JOHN L. Cox, a citizen of the United States, residing at Philadelphia, county of Philadelphia, and State of Pennsylvania, have invented a new and useful Improvement in Chromium-Steel Alloy, of which the following is a full, clear, and exact description.

The production of high chromium steel adapted to take a high polish and resist corrosion and to take and retain a cutting edge is well known. Such an alloy is especially adapted to the manufacture of cutlery and some of it makes an excellent non-deforming tool steel.

It has heretofore been supposed, by most metallurgists, that the percentage of carbon in such an alloy must be maintained relatively low. One patent places the upper limit of efficiency at .7 per cent. carbon with a preferential proportion of about .3 per cent. Another patent prescribes a wider range of from .1 to 1.0 per cent. Another patent, however, prescribes a relatively high carbon range of from 1. to 1.50 per cent. and states that for special uses the proportion of chromium may reach as high as 20 per cent., but in this patent the prescribed workable range of chromium is between 15 and 20 per cent. Still another patent describes an alloy consisting of chromium from 20 to 35 per cent., preferably from 25 to 30 per cent., but prescribes that the carbon content shall be from 1.5 to 3. per cent. Laboratory experimenters have tested ferrous alloys having various percentages of chromium and carbon and having usually, also, substantial percentages of other ingredients, without, however, arriving at any useful discovery of the superiority of any specific composition or the special availability of any specific composition for any particular use.

I have ascertained that in the manufacture of high carbon chromium alloy steels no imperative reason exists for restricting the percentage of chromium to below 20 per cent., which is the highest permissible percentage recognized by three of the above patents; but that, on the other hand, if the percentage of chromium be increased beyond twenty per cent., the percentage of carbon should be increased accordingly, but not

to the degree specified by the fourth patent mentioned. For example, if the percentage of chromium be just above twenty per cent., the percentage of carbon should not much exceed one per cent. With the highest practicable percentage of chromium the percentage of carbon should be less than the minimum (1.5), prescribed in the last named patent. While it may be possible to manufacture a serviceable chromium steel adapted for cutlery and having the property of resisting tarnishing and remaining bright, in which the percentage of carbon exceeds 1.5 per cent., the percentage of chromium, in such high carbon steel, must be raised so high that not only is the alloy relatively expensive but it becomes difficult to forge and impossible to roll to the thin sections required for cutlery.

I have made an excellent non-tarnishing cutlery steel having a carbon content of 1.15 per cent. and a chromium content of 23 per cent. The permissible range of carbon should not reach 1.5 per cent., and while the percentage of chromium is preferably not over 30 per cent., or thereabouts, it may be, without advantage, increased considerably beyond this percentage.

For some purposes a chromium-steel alloy containing between 1.0 and 1.5 per cent. of carbon, even though the percentage of chromium be relatively high, exhibits no advantage over an alloy containing correspondingly lower percentages of carbon and chromium. For other purposes, the marked tendency of high chromium steels to fail to harden on the surface can best be avoided by increasing the carbon content, while the objections to the higher carbon can be overcome by increasing the chromium content correspondingly.

Thus my discovery presents two aspects: First, that a high grade cutlery and tool chromium-steel alloy of a grade equal to such an alloy containing a relatively low percentage of carbon may be made with a percentage of carbon between 1.0 and 1.5 provided the percentage of chromium be increased above 20 per cent. Secondly, that such a relatively high carbon, high chromium, steel, when used for certain purposes, has advantages over a relatively low carbon

alloy, whatever the percentage of chromium in the latter may be.

A typical composition embodying my invention is the following:

Carbon ----- 1.15 per cent.  
Chromium --- 23 per cent.  
Iron----about 75 per cent.

My improved alloy is especially adapted to cutting purposes, as in the manufacture of machine tools for cutting metals and for table cutlery. It resists tarnishing, may be readily forged in the lower ranges, assumes a high degree of hardness on heating and quenching, and is readily softened by appropriate drawing methods.

While the ratio of carbon to chromium need not be invariable, inasmuch as a considerable excess of chromium is unobjectionable when the alloy is intended for certain uses, the ratio of chromium to carbon should be over 20:1 when the carbon content approximates the minimum range above specified, and should not be less than 15:1 when the carbon content is relatively high; while the ratio of chromium to carbon should not exceed 50:1 with a percentage of carbon close to the minimum range and should not exceed 40:1 with the highest permissible percentage of carbon.

With respect to the quality of stainlessness, comparing my improved alloy steel with the four compositions hereinbefore mentioned, only the two which require a low range of carbon are comparable with my product and I believe my product, in regard to this quality, is appreciably superior to any known composition. These two compositions, however, are not comparable with my composition with respect to the capacity to take and retain a cutting edge, while my composition, in this regard, is at least equal to the third of the compositions hereinbefore referred to. It is, of course, obvious that any composition having so high a carbon range as the fourth composition mentioned cannot be readily forged and cannot be readily softened. It will, therefore, be apparent that my product exhibits a very valuable union of qualities not heretofore known, namely: stainlessness, hot malleability and capacity for taking and holding a cutting edge and capacity for being readily softened for machining cold.

Having now fully described my invention,

what I claim and desire to protect by Letters Patent is:

1. A chromium-steel alloy containing over 1.0 per cent. and less than 1.5 per cent. of carbon and over 20 per cent. but less than 60 per cent. of chromium.

2. A chromium-steel alloy containing a preponderating proportion of iron, over 1.0 per cent. and less than 1.5 per cent. of carbon and over 20 per cent. and less than 30 per cent. of chromium.

3. A chromium-steel alloy containing over 1.0 per cent. and less than 1.5 per cent. of carbon and in excess of twenty per cent. of chromium wherein the ratio of chromium to carbon is between 15:1 and 50:1.

4. A chromium-steel alloy containing a predominating proportion of iron, carbon over 1.0 per cent. and less than 1.5 per cent. and chromium over 20 per cent., the same being readily forged, assuming a high degree of hardness on heating and quenching, being readily softened by drawing, and adapted to be made into a finished and highly polished cutting instrument resistive of corrosion and adapted to take on and retain a cutting edge.

5. An article of manufacture, such as cutlery and edged tools, composed of a steel alloy containing over 1.0 per cent. and less than 1.5 per cent. of carbon, over 20 per cent. of chromium and a preponderating proportion of iron.

6. A chromium steel alloy containing a preponderating proportion of iron, over 1.0 per cent. and less than 1.5 per cent. of carbon and in excess of twenty per cent. of chromium, wherein the ratio of chromium to carbon approximates 20:1.

7. A chromium steel alloy containing a preponderating proportion of iron, over 1.0 per cent. and less than 1.5 per cent. of carbon and in excess of twenty per cent. of chromium, wherein the ratio of chromium to carbon is not less than approximately 20:1.

8. A chromium steel alloy containing a preponderating proportion of iron, approximately 1.15 per cent. of carbon and approximately twenty-three per cent. of chromium.

In testimony of which invention, I have hereunto set my hand, at Philadelphia, Pa., on this 30th day of April, 1919.

JOHN L. COX.